

April 23, 1935.

J. C. SHERMAN

1,999,062

FIBER GEAR

Filed Aug. 23, 1932

Fig. 1.



Unimpregnated Disk  
Consisting of web of  
Interfeated wood pulp  
of high alpha cellulose content.

Fig. 2.



Disk impregnated  
with bakelite

Fig. 3.



Gear blank of superposed  
bakelite-impregnated disks  
bonded together.

Fig. 4.



Finished Gear

Inventor

John C. Sherman  
by Wright, Benson, Quincy & May

Attn:

## UNITED STATES PATENT OFFICE

1,999,062

## FIBER GEAR

John C. Sherman, Gorham, Maine, assignor to  
 Brown Company, Berlin, N. H., a corporation  
 of Maine

Application August 23, 1932, Serial No. 630,073

7 Claims. (Cl. 74—445)

This invention relates to the manufacture of so-called fiber gears, such as are frequently used when smooth and quiet performance is desired. In making such gears, it is sometimes the practice 5 to build up the gear blanks from plies of woven fabric, such as canvas, impregnated with suitable artificial resinous binders. One of the principal items of expense in such gears is the fabric base, which, however, has heretofore been found to be 10 an essential element in yielding an article of the desired strength, especially resistance to shock.

I have found that a refined or purified wood pulp of high alpha cellulose content may be advantageously used in an unwoven, comparatively 15 inexpensive form as the fibrous base in gears of the foregoing type, namely, in the form of a pre-fabricated web of interfelted fibers of such high porosity and absorptivity that it can be easily and perfectly impregnated throughout with the 20 proper artificial resinous binder and then be plied into a structure of the desired thickness.

It is essential that the pulp serving the purpose of the present invention be one refined to high alpha cellulose content, as the ordinary 25 wood pulps, such as sulphite and kraft, do not possess the desired absorptivity or other characteristics requisite to the securement of my base web. Such wood pulps as I employ as raw material are those which are arrived at only by refining the ordinary wood pulps to an alpha cellulose 30 content of at least about 93%, as by the reaction thereupon of caustic soda solutions or other alkaline liquors under special conditions, as now well-known in the pulpmaking industry. The 35 refined wood pulp is thus largely freed from less resistant cellulose, ligneous matter, resins, and other non-alpha cellulose components, which not only detract from its quality of absorptivity but render it unstable especially under the action of 40 heat.

The base web or felt answering my purposes is prepared in such a way that it possesses maximum porosity and absorptivity. This means that I depart from conventional papermaking 45 practice in fabricating the web. Indeed, rather than beating or hydrating the refined wood pulp to a marked degree, as is done in conventional papermaking practice, I employ a suspension of substantially unbeaten or unhydrated refined 50 wood pulp as the stock being sluiced to the headbox of the papermaking machine. The refined wood pulp can be handled in the form of an aqueous suspension without losing to any noteworthy extent its "free" condition, that is its 55 freedom from gelatinized or hydrated cellulose.

In this respect, refined wood pulp differs markedly from the ordinary wood pulps, which, in the presence of water, tend to generate mucilaginous hydrates which detract from the porosity and absorptivity of webs made therefrom, even when such ordinary wood pulps are used in substantially unbeatened condition. So, too, I handle my refined wood pulp on the papermaking machine in a way quite different from ordinary papermaking practice. Thus, I deposit the refined 10 wood pulp fibers in their free, substantially unbeatened condition on the usual wire cloth or screen of the papermaking machine into a web which is dewatered and dried without being subjected to the heavy pressures usually exerted on the web 15 by squeeze rolls or the like. As a result of such practice, I secure a fluffy web composed of loosely felted fibers and characterized by its extraordinary softness, porosity, and absorptivity.

On the accompanying drawing, Figures 1 to 20 4, inclusive, show in perspective the various stages of gear manufacture, beginning with an unimpregnated disk of the interfelted wood pulp and ending with a finished gear.

The dry, water-laid web may be died-out or 25 cut into disks which are to be impregnated and to constitute the plies of gear blanks. A disk in its unimpregnated and impregnated state is shown in Figures 1 and 2, respectively, a fragment of the disk being broken away for the sake 30 of clearer illustration. The disks may be impregnated with the desired, artificial resinous binder of the nature of bakelite. For example, they may be dipped into a 10% to 20% solution 35 of a bakelite varnish of about 60% solids content in a suitable solvent or thinner. At this concentration, the bakelite solution is thin and easy-flowing so that upon remaining immersed in the solution for about one-half to one minute, the disks become thoroughly impregnated with 40 the solution. They may then be squeezed to a bakelite solids content of, say, about 50%, based 45 on the weight of dry fiber. The impregnated disks may then be superposed into gear blanks of the desired thickness, which may be air-dried under heavy compression; and, when an air-drying bakelite varnish is employed, no heat treatment of the dried blanks is necessary. A gear blank of the desired character is illustrated in 50 Figure 3, this blank being of cylindrical form and designed more especially for cutting or shaping into a spur gear. If an "intermediate" type of bakelite varnish is used, the dried blanks should be heated or cured to render the varnish 55 infusible and insoluble and to impart other de-

sired characteristics thereto. The heat treatment or curing may be performed at a temperature and for a period of time consonant with the hardness desired in the finished article. For 5 instance, curing may be carried out in a press at a temperature of, say, 135° C. for about 90 minutes, under which conditions the plies become tenaciously bonded together and acquire 10 the hardness and hornlike toughness value in fiber gears.

Blanks produced in accordance with the foregoing method may undergo machining in the ordinary gear-shaping or gear-generating machines and be otherwise processed by the usual machines 15 employed in connection with metal gear blanks. For instance, the blank may be shaped and finished into a spur gear having the conventional form depicted in Figure 4. The finished gears are characterized by their homogeneity of structure 20 and the excellent resistance to shattering impact that comes with no local weak spots. It is by virtue of the character of the fiber used as raw material and of the web formed therefrom that the gears possess these desired properties, 25 for, if it be attempted to use ordinary paper webs, for instance, papers made from even high grade rags, as a material of construction for the gears, it is found that the gears are not proof against fracture and that they fail badly under the 30 stresses of use.

The manufacturing steps hereinbefore given are subject to considerable variation, but in any event the basic web should be made as hereinbefore described. As one possible modification, it 35 might be mentioned that the disks for building up the gear blanks may be died-out or cut from a web which has previously undergone impregnation with the desired artificial resinous binder. Thus, the web as it comes in dry condition 40 from the web-forming machine may be impregnated with a bakelite varnish of the intermediate type, then dried, and, if desired, accumulated as rolls. Disks of the desired size may then be died-out or cut from the impregnated 45 sheet, stacked into gear blanks of the desired thickness, and the blanks compressed at elevated temperature to cause their plies to unite as well as to transform the bakelite to the desired hard, non-frangible, insoluble and infusible 50 condition.

The term "bakelite" is used in the foregoing description and in the appended claims in its comprehensive sense to include the various phenol and/or aldehydic or other artificial resinous condensation products, which, in their ultimate or cured condition, are comparatively 55 hard, non-frangible, insoluble, and infusible.

I claim:

1. A gear made up of compressed, plied, water-laid webs of loosely felted wood pulp having an alpha cellulose content of at least about 93% and impregnated substantially uniformly throughout and bonded together with an artificial, resinous binder of the nature of bakelite.

2. A gear made up of compressed, plied, water-laid webs of loosely felted, substantially unbeaten, cellulose pulp having an alpha cellulose content of at least about 93% and impregnated substantially uniformly throughout and bonded together with a cured, artificial, resinous binder of the nature of bakelite.

3. A gear made up of compressed, plied, water-laid webs of loosely felted, substantially unbeaten, wood pulp having an alpha cellulose content of at least about 93% and impregnated substantially uniformly throughout and bonded together with a cured, artificial, resinous binder of the nature of bakelite in the amount of about 50% by weight of the pulp.

4. A gear made up of plied, waterlaid webs of substantially unhydrated, interfelted cellulose fiber of high alpha cellulose content and in themselves of high porosity and absorptivity but impregnated substantially uniformly throughout and bonded together with a binder of the nature of bakelite, rendering said gear structure highly resistant to shattering upon impact and to the 3 stresses of use.

5. A gear made up of plied, waterlaid webs of substantially unhydrated, interfelted cellulose fiber having an alpha cellulose content of at least about 93% and in themselves of high porosity and absorptivity but impregnated substantially uniformly throughout and bonded together with a binder of the nature of bakelite, rendering said gear structure highly resistant to shattering upon impact and to the 4 stresses of use.

6. A gear made up of compressed, plied, waterlaid webs of loosely felted cellulose pulp having an alpha cellulose content of at least about 93% and impregnated substantially uniformly throughout and bonded together with a binder 4 imparting thereto the qualities of hardness and hornlike toughness.

7. A gear made up of compressed, plied, water-laid webs of felted, substantially unbeaten wood pulp having an alpha cellulose content of at 5 least about 93% and impregnated substantially throughout and bonded together with a binder imparting thereto the qualities of hardness and hornlike toughness.

JOHN C. SHERMAN. 5